

# UNITED STATES PATENT OFFICE.

ALLEN ROGERS, OF BROOKLYN, NEW YORK.

## PROCESS OF MAKING LEATHER.

1,346,385.

Specification of Letters Patent. Patented July 13, 1920.

No Drawing.

Application filed May 5, 1920. Serial No. 379,050.

To all whom it may concern:

Be it known that I, ALLEN ROGERS, a citizen of the United States, residing at Brooklyn, in the county of Kings and State of New York, have invented certain new and useful Improvements in Processes of Making Leather, of which the following is a specification.

This invention relates to processes of making leather; and it comprises a process of making leather or tanning hides wherein the hides are first treated with an aluminum compound containing alumina in such a state as to render it capable of being taken up and are thereafter treated with shark liver oil; all as more fully hereinafter set forth and as claimed.

In the manufacture of leather from hides, cod liver oil is sometimes used; the skins being milled or worked with such cod liver oil and then packed down in boxes to oxidize; or hung up in hot rooms to the same end. Some such means are necessary to initiate and continue oxidation; and in practice it is found that several repetitions of the process are necessary before the skins are thoroughly tanned. I have found that by using shark liver oil I can much abbreviate the operation; that with shark liver oil oxidation is initiated and continued without the usual packing down or hanging in hot rooms. The oxidation is also much more thorough and I can secure results in a single operation with shark liver oil which with cod liver oil require several.

In the present invention I utilize this fact in a particular manner; utilizing the leather making properties of shark liver oil in a tannage process. In this process I first submit the skins to an alum tannage, dry the treated skins thoroughly and, after drying, bring to a sammied or semi-moist condition with water and mill the stock with shark liver oil from 2 to 3 hours. During this milling process, the alum-treated stock absorbs the shark liver oil and becomes more or less hot in the drums. The oil may be applied during the drumming operation instead of preliminarily thereto. When the

stock has been thoroughly saturated with oil, it is simply hung up in drying rooms. During this hanging thorough oxidation takes place and the tannage is completed. After the hides or skins become of a dry consistency they can be dampened again with water, oiled off with tallow or other mixture, set out and finished in the usual manner.

In the alum tanning stage, the hides may be submitted to a single or double bath containing sulfate of alumina or alum with chemicals adapted to convert the alumina into a condition in which it can be adsorbed by the hide. Any mildly alkaline material, such as soda, borax, sodium phosphate, etc., may be employed as such a chemical, either together with aluminum sulfate (sulfate of alumina) in a single bath process or subsequently thereto as in a 2-bath process.

In the first stage of the operation, in lieu of performing a mineral tannage with alumina (aluminum sesquioxid), other equivalent bases, such as chrome (chromium sesquioxid), or iron (iron sesquioxid) may be used.

In a general way, I have found that shark liver oil is, because of its quickly oxidizing properties, peculiarly advantageous in performing an oil treatment subsequent to a preliminary tannage with other materials. It is, for example, particularly advantageous in stuffing ordinary belt leather, harness leather and latigo leather and also as a fat liquoring oil for light leather. It is useful in the manufacture of chamois skin and glove leather.

In the described treatment using shark liver oil it is not necessary to add oxidizing catalysts of any kind, although of course this may be done.

What I claim is:

1. In the conversion of hides and skins into leather, the process which comprises submitting the material to a mineral tanning operation and then to a treatment with shark liver oil.
2. In the conversion of hides and skins into leather, the process which comprises

submitting the material to a mineral tanning operation with a sesquioxid and then to a treatment with shark liver oil.

3. In the conversion of hides and skins into leather, the process which comprises submitting the material to a mineral tanning operation with alumina and then to a treatment with shark liver oil.

4. In combination tannage processes, the method which comprises saturating a partially tanned hide or skin with shark liver oil and oxidizing such oil by a simple hanging operation. 10

In testimony whereof, I affix my signature hereto.

ALLEN ROGERS.